

## UNITED STATES PATENT OFFICE

2,363,904

## PROCESS FOR DYEING TEXTILE FIBERS

Chiles Emory Sparks and Joseph Francis Laucius,  
Wilmington, Del., assignors to E. I. du Pont de  
Nemours & Company, Wilmington, Del., a cor-  
poration of Delaware

No Drawing. Application December 31, 1942,  
Serial No. 470,836

10 Claims. (Cl. 8—42)

This invention relates to an improved process for dyeing textile materials. More particularly, this invention is concerned with that mode of dyeing wherein textile fibers, for instance cellulose fiber, wool, cellulose esters or nylon, are impregnated with water-soluble azotized polyamino-phthalocyanines and then treated further in any one of a number of optional methods to develop on the fiber various shades of good fastness properties.

It is an object of this invention to improve the affinity of the fiber for the azotized polyamino-phthalocyanine compound, whereby to obtain stronger dyeings on the fiber while using relatively weak impregnation baths. It is a further object of this invention to provide an improved method of procedure whereby the impregnation bath, which is generally an aqueous solution of the azotized polyamino-phthalocyanine compound, shall become substantially exhausted of color in the dyeing, thus increasing the general economy of the process. Other and further important objects of this invention will appear as the description proceeds.

In this specification and in the claims below the term azotized is used as a generic term for the common expressions "diazotized," "tetrazotized" and "polydiazotized." In other words, it is intended to describe the state of a substance or the process wherein one or more amino groups have been converted into diazonium groups, the prefixes di-, tetra- or polydi- being dropped off to avoid confusion.

In British Patent No. 535,935 is disclosed a process of dyeing textile materials by impregnating the same with an aqueous solution containing azotized tetra-amino-phthalocyanines, and then treating the fiber to develop the color on the fiber. Two modes of development are therein described. In one of these, the impregnated fiber is treated under conditions which result in decomposition of the diazonium groups, producing on the fiber fast colors of the phthalocyanine series. The conditions generally involve heating in the presence of water or steam alone, in the presence of aliphatic alcohols, or in the presence of aqueous solutions of substances which are not generally coupling components for the production of azo dyes. The resulting color on the fiber is therefore not an azo dye. In the other method, development is effected at moderate temperature, say 0° to 30° C., that is, a temperature less than that which would decompose the diazo groups, but the treatment bath contains an azoic coupling component, whereby coupling takes place in regu-

lar fashion and a water-insoluble azo color of the phthalocyanine series is produced on the fiber.

According to latest developments in this field (which constitute subject matter of a patent application by James William Libby, Jr., Serial No. 471,731), development on the fiber may also be achieved by reaction with coupling components which possess water-solubilizing groups; for instance, the naphthol-sulfonic acids, the amino-naphthol-sulfonic acids, the aryl-pyrazolone-carboxylic acids, the sulfo-aryl-pyrazolones, and other similar components which are generally considered as outside the class of azoic coupling components; and there results on the fiber nevertheless a dyeing of satisfactory fastness qualities. In still another process, the developed dyeing on the fiber is further developed by treatment with metallizing agents which further modify or improve its fastness qualities or shade.

Again, according to copending application Serial No. 443,668 by N. H. Haddock (Patent No. 2,349,090, issued May 16, 1944), it is possible to color fabric either by padding it with an aqueous bath or by printing it with a printing paste containing a stabilized modification of an azotized polyamino-phthalocyanine, and then treating the fabric by various methods to develop the color on the fiber. Several different modes of stabilization of the diazo group have been mentioned and discussed in said application, but the process of applying them to the fiber is essentially the same, as outlined generally above.

All the above processes have the two essential features in common that the fiber is impregnated first with an azotized polyamino-phthalocyanine, and that it is then subjected to treatment which develops the color on the fiber. And in all of these, the efficiency of the process and the strength of the resulting dyeing will naturally depend on the degree of adsorption of the azotized compound onto the fiber in the first step of the process. Unfortunately, this degree is not very high, due to the relatively poor affinity of azotized polyamino-phthalocyanines for cellulosic fiber. As a result, strong dyeings are not obtainable unless concentrated padding baths are employed, and the exhaustion of color in these baths is unsatisfactory. In the case of azotized copper-tetra-amino-phthalocyanine, for instance, when applied without the aid of the special pre-treatment of this invention, a highly concentrated solution of the tetradiazonium compound must be used to get strong dyeings, and the exhaustion is poor.

We have now found that the affinity of textile

fiber for azotized polyamino-phthalocyanines may be considerably increased, sometimes several fold, and that strong dyeings after the eventual development may be obtained, if the fabric is pretreated or mordanted, so to speak, with an aqueous bath containing a water-soluble heteropoly compound, or the acid or water-soluble salt-form of the heavy metal constituent of a heteropoly acid; in other words, vanadic, molybdc or tungstic acids and their salts. Our novel process of dyeing therefore comprises the steps of impregnating the textile material, for instance cotton, wool, cellulose acetate or nylon, with an aqueous bath containing heteropoly acids or derivatives thereof, entering the textile into a solution of an azotized amino-phthalocyanine, working the goods until the solution is well exhausted of its soluble azotized product, and finally fixing or developing the dyed textile with various agents or under various conditions, as hereinabove mentioned, to cause the diazonium groups to be decomposed, exchanged, reduced or coupled, yielding the desired shade of dyeing. In this manner, strengths many times greater than those of British Patent No. 535,935 are obtained; moreover, the azotized phthalocyanine can be exhausted from the dyebath.

Heteropoly compounds include those acids and salts which contain acid anhydrides of one or more elements combined with a hydrate or salt of the acid of another element. (Text Book of Inorganic Chemistry, edited by J. Newton Friend, vol. VII, part III, page 163. Other definitions may be found in Text Book of Inorganic Chemistry by Fritz Ephraim; translated by Thorne, London, 1926, pages 405-415; also, Systematic Inorganic Chemistry by Caven and Lander, London, 1932, page 327.) The heteropoly acids generally contain the anhydride of a heavy metal from the 5th or 6th group of the periodic system, more especially vanadium, molybdenum or tungsten, and are typified further by the following examples which we have found useful for our invention: phospho-molybdc acid, phospho-tungstic acid, phospho-molybdo-tungstic acid, phospho-vanadic acid, silico-tungstic acid, boro-tungstic acid, silico-molybdc acid and boro-molybdc acid. The acids or salts of the heavy metal constituent of the hetero-poly acid may be used also, for example sodium molybdate, sodium tungstate, tungstic acid, etc. These compounds may be applied to the textiles as free acids or as the alkali metal salts or as a mixture of free acids or a mixture of salts, as for example, a mixture of disodium hydrogen phosphate and sodium tungstate or a mixture of disodium hydrogen phosphate and sodium molybdate. The quantities of these agents in the pre-treatment bath may be varied within wide limits, for instance from 0.1 to 2.5 parts by weight per 100 parts by weight of textile material to be treated.

As a further feature of our invention, the textile fiber may be further treated, prior to dyeing with the diazo compound, with agents adapted to fix the heteropoly acids on the fiber by lowering their solubility. Suitable agents for this purpose are water-soluble ammonium salts, quaternary ammonium compounds and water-soluble guanidine derivatives, as typified by ammonium chloride, guanidine carbonate, cetyl pyridinium bromide, octadecyl pyridinium bromide, and beta-ureido-ethyl-pyridinium chloride. The amounts of these auxiliary agents used in this fixing treatment may likewise vary within wide limits; say,

from 0.1 to 1.5% based on the weight of the textile material treated.

As for the azotized polyamino-phthalocyanines to which our invention is applicable, these may be any of those hitherto mentioned in the art for this purpose. For instance, they may be derived from copper-tetra-(4)-amino-phthalocyanine, copper-tetra-(3)-amino-phthalocyanine, copper-triamino-phthalocyanine, copper-diamino-phthalocyanine and the corresponding polyamino derivatives of nickel-phthalocyanine, cobalt-phthalocyanine or dihydrogen-phthalocyanine ("metal-free" phthalocyanine). The amino-phthalocyanine is azotized in the usual manner with sodium nitrite and mineral acid, and the padded cloth is passed through the solution until the desired strength is attained or until the soluble diazonium compound is exhausted. Alternatively, an aqueous solution of a stabilized form 20 of the polydiazonium phthalocyanine compound, for instance the zinc chloride double salt, may be employed as impregnation bath.

The development of the color on the fiber may be effected in any one of the various methods 25 aforementioned and may include for instance:

I. Treatments designed to decompose the diazonium groups, or to replace them by radicals which are not in the class of coupling components. Agents suitable for this purpose are: 30 water, methyl alcohol, ethyl alcohol, ethylene glycol, diethylene glycol, ethylene-glycol-mono-methyl-ether, sodium sulfide, pyridine, sodium carbonate, ammonia, potassium dichromate, sodium hypophosphite, potassium iodide, potassium bromide, cuprous chloride, sodium thiosulfate, and glucose, either at ordinary or raised temperatures.

II. Treatment with aqueous baths containing coupling components, for instance:

(a) Coupling compounds containing reactive methylene groups, such as the pyrazolones, aryl pyrazolones, aryl pyrazolone carboxylic acids, dimethyl-dihydro-resorcinol, acetyl acetone, acetacet arylides, and barbituric acid;

(b) Ice color coupling components (so-called azoic coupling components), such as alpha- and beta-naphthol, the naphthol-carboxylic acids, and the arylamides of 2,3-hydroxy-naphthoic acid;

(c) Various other coupling components, such as the phenols, carboxy-phenols, naphthol-sulfonic acids, naphthol-disulfonic acids, naphthol-trisulfonic acids, amino-naphthol-sulfonic acids, amino-naphthol-disulfonic acids, amino-naphthols, amino-naphthalene-sulfonic acids, hydroxy-quinolines, resorcin, meta-phenylene-diamine; and

(d) Mixtures of any of the above. A variety of shades may be obtained, as will be further shown by the following examples which are given to illustrate the invention without any intent to limit it. Parts mentioned are by weight.

#### Example 1

05 Cotton cloth (180 parts) is prepadded with a solution containing 2.55 parts sodium tungstate, 0.5 part disodium hydrogen phosphate and 6 parts concentrated hydrochloric acid (37%) in 500 parts water and passed through a wringer set so that 180 parts of solution are retained by the cloth.

The cotton cloth, prepadded as above, is then passed through a solution of tetradiazotized copper-tetra-(4)-amino-phthalocyanine, made by azotizing 1.8 parts of copper tetra-(4)-amino-

phthalocyanine with 60 parts concentrated hydrochloric acid (37%), 9.5 parts of 2-normal sodium nitrite and ice to maintain the temperature at 0-10° C. and diluting to 1800 parts with water. When the soluble diazonium compound has been exhausted, the cloth is rinsed in cold water. The cloth from the preceding treatment is then passed through boiling water. A strong green dyeing which is extremely fast to light, washing and weathering is obtained.

If ethyl alcohol at 70° C., ethylene glycol at 100° C., or diethylene glycol at 100° C. is substituted for the boiling water, a strong, bright blue dyeing, extremely fast to light, washing and weathering is obtained.

*Example 2*

Cotton sheeting (180) parts) is prepped with a solution containing 3.9 parts sodium molybdate, 0.44 part disodium hydrogen phosphate and 6 parts concentrated hydrochloric acid in 500 parts water, and then passed through a wringer set so that 180 parts of solution are retained by the cloth. The sheeting is then passed through a solution containing 20 parts ammonium chloride in 400 parts water and then passed through the wringer so that 180 parts of solution are retained by the cloth. The cloth is then impregnated with azotized tetramino-copper-phthalocyanine as in Example 1. The rinsed cloth is passed through a 5% aqueous solution of 1-(4'-sulfo-phenyl)-3-methyl-5-pyrazolone containing 5% sodium carbonate. There is obtained a green dyeing fast to light and washing.

In the place of 1-(4'-sulfo-phenyl)-3-methyl-5-pyrazolone, the following reagents may be substituted to give the shades listed below:

|    | Reagent                                                                                          | Shade         |
|----|--------------------------------------------------------------------------------------------------|---------------|
| 1  | 2-naphthol                                                                                       | Dull violet.  |
| 2  | 1-naphthol-4-sulfonic acid                                                                       | Do.           |
| 3  | Salicylic acid                                                                                   | Blue green.   |
| 4  | Ethyl-aceto-acetate                                                                              | Bright green. |
| 5  | 8-hydroxy-quinoline                                                                              | Grey.         |
| 6  | 1-amino-8-naphthol-2,4-disulfonic acid                                                           | Blue grey.    |
| 7  | 1-naphthol-3,8-disulfonic acid                                                                   | Do.           |
| 8  | 1,8-dihydroxy-naphthalene-3,6-sulfonic acid                                                      | Do.           |
| 9  | Acetyl acetone                                                                                   | Bright green. |
| 10 | 3-methyl-5-pyrazolone                                                                            | Green.        |
| 11 | Dimethyl-dihydro-resorcinol                                                                      | Bright green. |
| 12 | Barbituric acid                                                                                  | Do.           |
| 13 | 2,4-dihydroxy-quinoline                                                                          | Green.        |
| 14 | 2-phenyl-amino-5-naphthol-7-sulfonic acid                                                        | Grey.         |
| 15 | 1-naphthylamine-6-sulfonic acid                                                                  | Do.           |
| 16 | Iophorone                                                                                        | Blue green.   |
| 17 | Aceto-acet-p-phenetidine                                                                         | Green.        |
| 18 | 1-phenyl-3-methyl-pyrazolone                                                                     | Do.           |
| 19 | Anilide of 2-oxo-3-naphthoic acid                                                                | Dull violet.  |
| 20 | Resorcin                                                                                         | Dull brown.   |
| 21 | meta-Phenylene-diamine                                                                           | Brown.        |
| 22 | Mixture of three parts 1-(4'-sulfo-phenyl)-3-methyl-pyrazolone and one part m-phenylene-diamine. | Black.        |
| 23 | Mixture of one part m-phenylene-diamine and one part ethyl aceto-acetate.                        | Do.           |

*Example 3*

Cotton cloth (10 parts) prepped as in Example 1 is passed through a solution of tetra-diazotized copper-tetra-(4)-amino-phthalocyanine made by dissolving 0.5 part of the zinc chloride tetra-diazo salt of copper-tetra-(4)-amino-phthalocyanine in 400 parts of water. The dyeing is treated with boiling ethyl alcohol to produce a blue dyeing which is fast to light, weathering and washing.

*Example 4*

Cloth prepped and impregnated as in Example 1 is passed into a boiling 5% solution of sodium hypophosphite. A green-blue dyeing having excellent fastness to light, weathering, and washing is obtained.

If, in place of the boiling sodium hypophosphite solution, there are used the following reagents, the following shades are obtained: (Throughout this example and the next following, wherever solutions are named, unless otherwise specified, aqueous solutions are implied.)

|    | Reagent                            | Shade       |
|----|------------------------------------|-------------|
| 10 | 1 5% potassium iodide solution     | Green.      |
|    | 2 5% potassium bromide solution    | Do.         |
|    | 3 5% pyridine                      | Do.         |
|    | 4 5% sodium sulfide solution       | Do.         |
|    | 5 5% formaldehyde solution         | Blue green. |
|    | 6 5% formic acid solution          | Do.         |
|    | 7 Isoamyl alcohol                  | Blue.       |
| 15 | 8 2% potassium dichromate solution | Dull green. |

*Example 5*

Cloth prepped with 0.5% phosphomolybdcic acid according to the procedure set forth in Example 1 is passed through an azotized solution of copper-tri-(4)-amino-phthalocyanine made from 1.2 parts copper tri-(4)-amino-phthalocyanine, 24 parts concentrated hydrochloric acid, 4 parts of 2-normal sodium nitrite, 300 parts of water, and ice to bring the temperature to 0-5° C. for one hour. The dyeing thus obtained is three times as strong as one in which no prepadding agent is used.

The dyed textile is then passed into a 5% solution of acetyl acetone to which 5% sodium carbonate was added. A bright yellow green dyeing having good washing and light fastness is obtained.

If in the above example, acetyl acetone is replaced by other reagents, the following shades are obtained:

|    | Reagent                                     | Shade        |
|----|---------------------------------------------|--------------|
| 40 | 1 1-(4'-sulfo-phenyl)-3-methyl-5-pyrazolone | Green.       |
|    | 2 2-naphthol-3,6-disulfonic acid            | Dull violet. |
|    | 3 2-amino-5-naphthol-7-sulfonic acid        | Black-brown. |

*Example 6*

The dry zinc chloride tetradiazo salt from 6.35 parts of copper tetra-(4)-amino-phthalocyanine is slurried in 100 parts of ethyl alcohol at 25-30° C. for ten minutes and then filtered, washed with dry acetone and dried. A blue product which is soluble in water is obtained. When applied to cotton pretreated in the manner set forth in Example 1 and then after-treated with boiling water, it gives a bright blue dyeing. If boiling ethyl alcohol is substituted for boiling water, a redder shade blue is obtained.

*Example 7*

Five parts of cotton cloth were prepped with 5 parts of a 1% solution of silico tungstic acid and the padded cloth was entered into a solution of azotized copper-tetra-(4)-amino-phthalocyanine. The dyeing showed approximately five times the strength over the dyeing of an unprepadded cloth treated in the same manner. The dyeing was treated with boiling water to give a green dyeing of excellent fastness to light and washing.

If in place of silico tungstic acid, sodium molybdate or a mixture of sodium molybdate, sodium tungstate and sodium phosphate is used, a dyeing of similar properties is obtained.

*Example 8*

Viscose rayon is prepped and impregnated as in Example 1. The impregnated fiber is passed

into boiling water. A green dyeing fast to light and to washing is obtained.

*Example 9*

Wool is preadded and impregnated as in Example 1, and the treated material is steamed for five minutes. The resulting green dyeing shows excellent fastness to light.

In the above examples, in lieu of the freshly prepared solutions of the azotized polyamino-phthalocyanines, solutions of the corresponding zinc-chloride double-salts may be employed; and vice versa. Likewise, in any of the above examples where a metallizable azo dye is produced on the fiber, for instance an azo dye containing OH groups ortho to the azo groups or OH groups ortho to carboxylic acid groups, the fiber may be after-treated with azo-dye metallizing agents, for instance, water-soluble salts of copper, nickel, chromium or cobalt, as more fully described and claimed in copending applications of Libby and Woodward, Ser. No. 471,730, and of Rossander, Libby and Woodward, Ser. No. 471,732.

Many other variations in details may be practiced with our invention, as will be readily apparent to those skilled in this art.

We claim:

1. In the process of padding textile material with a member of the group consisting of polydiazonium compounds of the phthalocyanine series and stabilized forms of said polydiazonium compounds, the improvement which consists of pretreating the fabric with a reagent selected from the group consisting of molybdic acid, tungstic acid, vanadic acid, heteropoly acids derived from said acids, and the water-soluble salts of any of these acids, whereby to increase the affinity of the textile material for said polydiazonium compounds.

2. A process as in claim 1, wherein the textile material is further treated with a water-soluble chemical compound containing pentavalent nitrogen and adapted to fix said pre-treating agents onto the fiber by lowering the solubility thereof, prior to treatment with said polydiazonium compounds.

3. A process as in claim 1, wherein the textile material is further treated with an agent selected from the group consisting of water-soluble ammonium salts, quaternary ammonium compounds and water-soluble guanidine salts, prior to treatment with said polydiazonium compounds.

4. A process for dyeing textile fiber, which comprises subjecting said fiber to a treatment which includes the step of impregnating said fiber with a compound selected from the group consisting of molybdic acid, tungstic acid, vanadic acid, heteropoly acids containing the nucleus of at least one

of said acids, and water-soluble salts of any of the acids aforementioned, whereby to increase the affinity of the textile material for diazonium derivatives of phthalocyanine compounds; then impregnating said textile material with an azotized form of a polyamino-phthalocyanine compound; and thereafter subjecting the impregnated fiber to treatment adapted to develop the color on the fiber.

5. A process as in claim 4, wherein the treatment in the last mentioned step includes action upon the fiber with agents adapted to eliminate nitrogen from the diazonium groups on the fiber, whereby to produce a water-insoluble dyestuff on the fiber.

6. A process as in claim 4, wherein the treatment in the last mentioned step comprises treatment of the fiber with coupling components adapted to produce an azo dye on the fiber.

7. A process for dyeing textile fiber, which comprises subjecting said fiber to a treatment which includes the step of impregnating said fiber with a compound selected from the group consisting of molybdic acid, tungstic acid, vanadic acid, heteropoly acids containing the nucleus of at least one

of said acids, and water-soluble salts of any of the acids aforementioned, whereby to increase the affinity of the textile material for diazonium derivatives of phthalocyanine compounds; then impregnating said textile material with an azotized form of copper-tetramino-phthalocyanine; and thereafter subjecting the impregnated fiber to treatment adapted to develop the color on the fiber.

8. A process as in claim 7, wherein the treatment in the last mentioned step consists of heating the impregnated fiber in contact with a liquid selected from the group consisting of water, aliphatic alcohols, and aqueous solutions of reagents which facilitate the elimination of nitrogen from the diazonium groups on the fiber.

9. A process as in claim 7, wherein the treatment in the last mentioned step consists of impregnating the fabric with reagents adapted to act as coupling components for the diazonium groups, whereby to develop an azo dyestuff on the fiber.

10. A process as in claim 7, wherein the fiber after the first mentioned impregnation and prior to impregnation with an azotized form of said color is further treated with a member of the group consisting of water-soluble ammonium salts, quaternary ammonium compounds and water-soluble guanidine salts, whereby to fix on the fiber the reagents employed in the first mentioned treatment.

CHILES EMORY SPARKS.  
JOSEPH FRANCIS LAUCIUS.